# EUROPEAN PATENT SPECIFICATION

(11) **EP 0 105 730 B1**
(45) Date of publication and mention of the grant of the patent: **09.08.1989**
(21) Application number: 83305892.8
(22) Date of filing: 29.09.1983
(51) Int. Cl.: D04H 1/54

(54) **Open mesh belt bonded fabric**
Durch offenmaschiges Band gebundener Stoff
Etoffe liée par courroie à mailles ouvertes

(30) Priority: 30.09.1982 US 430310
(43) Date of publication of application: 18.04.1984
(73) Proprietor: CHICOPEE, New Brunswick New Jersey 08903 (US)
(72) Inventor: Cancian, Annamaria Cesco, Plainsboro New Jersey 08536 (US); Shimalla, Charles J., Kendall Park New Jersey 08824 (US)
(74) Representative: Jones, Alan John

(56) References cited:
- DE-A- 2 644 961
- GB-A- 1 189 851
- US-A- 3 616 031
- US-A- 4 068 036
- US-A- 4 103 058

## Description

### Background of the invention

Method and apparatus for drying and heat setting fibrous webs are known. One such method and apparatus is set forth in U.S. 3,442,740. The apparatus described comprises the rotating heated roll and flexible endless restraining belt which travels around the roll. A web is inserted between the belt and the roll. In the modification described in this patent, the web travels around the roll under the restraining belt. The web is doffed from the heating roll onto the belt which transports it to a cooling roll. The web travels around the cooling roll while under the restraining belt and is then doffed from the roll and the belt.

In the commercially available Honeycomb Dryer, a fibrous web is passed around a for- maminous roll while being subjected to forced air heat directed toward the outside surface of the roll. This apparatus, although originally used for drying fibrous webs, has been suggested for use in fusing fibrous webs comprising thermoplastic materials. One modification of the apparatus and method comprises the use of a restraining belt extending about the roll, which belt is laid down atop the fibrous web to restrain the web against the surface of the roll during the bonding or drying process. The foraminous surface of the roll creates a smooth fabric face. In the method and apparatus of the present invention, an open mesh network is disposed about the surface of the roll or substituted for the surface of the roll. The open mesh network surface molds the fabric creating a puffed surface.

Our copending European Patent Application EP-A-0106604, filed contemporaneously herewith discloses the use of an open mesh belt as a restraining belt in the Honeycomb dryer. That application also discloses the use of an open mesh belt adjacent a web and between two carrier belts. The fabrics formed have a patterned surface formed by the tension of the open mesh belt against the web during bonding of the fabric. The fabrics have good strength and high loft.

### Summary of the invention

The present invention comprises an apparatus, method and fabric formed thereby for thermal bonding a web comprising at least 10 percent conjugate fibers. In the apparatus of the present invention, an open mesh network comprises or is superimposed on a moving surface such as a rotating drum and a source of forced heated air is directed toward the open mesh network. In the method of the present invention, a fibrous web comprising conjugate fibers comprising a low melting point thermoplastic component is fed to and superimposed over the open mesh network rotating on the rotating drum. Forced heated air impinging on the web molds the web and puffs the fibers out of the plane of the fabric into the open areas of the open mesh network and fuses the low melting point component of the conjugate fibers in the web. The fabric formed thereby is a very high loft fabric having patterned puffed regions on one surface thereof. The method of the present invention may also be practiced using a restraining belt causing regions of densification between the puffed regions. The use of a conventional smooth surfaced restraining belt compresses the web against the open mesh structure creating regions of densification between the puffed regions of the fabric and a smooth surface on the opposite side of the fabric. If the restraining belt is formed of another open mesh network, it will create densified regions as above, and will create a pattern of embossed type densified regions on the surface of the fabric opposite the puffed surface.

### Brief description of the drawings

Figure 1 is a schematic side view of an apparatus according to the present invention;
Figure 2 is a perespective view of a portion of an open mesh network for use in the apparatus and method according to the present invention;
Figure 3 is a perspective view of one embodiment of a fabric formed according to the method of the present invention;
Figure 3A is a fragmentary section of the fabric of Figure 3 illustrating schematically how the fabric is formed;
Figure 4 is a perspective view of another embodiment of a fabric formed according to the present invention;
Figure 4A is a fragmentary section of the fabric of Figure 4 illustrating schematically how the fabric is formed;
Figure 5 is a perspective view of another embodiment of the fabric formed according to the . method of the present invention; and
Figure 5A is a fragmentary section of the fabric of Figure 5 illustrating schematically how the fabric is formed.

### Detailed description of the drawings

Figure 1 illustrates schematically and in cross- section an apparatus according to the present invention. In the preferred embodiment shown, the apparatus comprises a framework shown generally at 10 with a movable surface comprising in this embodiment a rotatable drum 12. The apparatus had heating means (not shown) within the frame at 14. The heating means directs forced heated air onto the outside of the movable surface. Though it is not necessary that the path of the movable surface comprise a curve when as in this embodiment, when it does, it is preferred to exhaust the confluence of forced air by drawing a vacuum from a point within the curve. Most preferably the force of the impinging air and the vacuum are balanced, which balance is dependent on the web being processed.

In the improved apparatus of the present invention, an open mesh network 16 is superimposed on the movable surface. The open mesh network may comprise an endless belt as shown, which extends away from the roll 12 and is transported back to the roll by means 18,20, and 22 for moving an endless belt open mesh structure to and from the movable surface. In an alternate embodiment, the open mesh network may be wound tightly about just the drum. In still another alternative, the open mesh network may be used to form the surface of the drum or movable surface. In the preferred embodiment shown, the endless belt open mesh network has two advantages. The endless belt open mesh network may be used to transport the web to a cooling station as will be described later; and may be easily replaced by another open mesh network of different configuration.

A portion of an open mesh structure for use in the apparatus and method according to the present invention is shown at 40 in Figure 2. The open mesh structure has open areas 42 and also has a depth 44. In the method according to the present invention, a web 24 comprising at least 10 percent conjugate fibers is disposed across a moving open mesh structure surface and the exposed side of the fabric is then subjected to forced heated air. The fibers disposed across the open areas 42 are bent out of the plane of the web and into the open regions by the forced heated air thereby creating a fabric having a pattern of puffed regions of lesser density than the overall fabric created by the fibers bent out of the flame of the fabric. The forced heated air also heats and fuses the low melting point component of the conjugate fibers of the web to fibers in the web. The apparatus of the present invention may also comprise a cooling station (not shown) at 26 which in its preferred embodiment comprises forced cooled air. In a still preferred embodiment, the means for carrying the endless belt open mesh away from the drum may. comprise means for carrying the open mesh network into the cooling station.

Figure 3 depicts a fabric formed according to the present invention. The fabric shown generally at 50 has a very high loft and low density. One face 52 of the fabric comprises a pattern of puffed regions 54 wherein the fibers are bent out of the.plane 55 of the fabric. As shown in Figure 3A, these puffs are formed in the open areas 42 of the open mesh structure by the forced heated air. These puffed regions have lower density than the overall fabric. The other surface 56 of the fabric may have a pattern of recesses 58 corresponding to the puffed regions 54. At lower air velocities, the fabric formed has a substantially uniform density throughout, with puffed regions and recesses being matched to give a molded fabric wherein the entire fabric is moved into the open areas, 42, of the open mesh structure.

In a preferred construction, the nonwoven fabrics of the present invention are made from polyester/polyethylene conjugate fibers wherein at least about 50 percent of the surface of the individual fibers is polyethylene. It is preferred to employ sheath/core fibers with the polyethylene as the sheath and the polyester as the core. Either eccentric or concentric sheath/core fibers can be employed. The fibers will usually have a denier within the range of from about 1 to about 6 (about 1.111 to about 6.666 dtex), and are in excess of about 1/4-inch (6.35 mm) in length, up to about 3 or 4 inches (7.6 or 10.2 cm) long.

Preferably, the conjugate fibers employ high density polyethylene, that is, linear polyethylene that has a density of at least about 0.94, and a Melt Index <"M.).") by ASTM D-1238 (E) (190°C., 2160 gms.) of greater than 1, preferably greater than about 10, and more preferably from about 20 to about 50. Usually the fibers will be composed of about 40 to 60 weight percent, and preferably 45 to 55 weight percent, polyester, the remainder being polyethylene.

A minor proportion of other fibers, preferably nonabsorbent staple fibers such as polyester fibers, can be used along with the polyester/ polyethylene conjugate fibers.

The fabrics of the invention are produced byfirst forming a fibrous web comprising a loose array of the conjugate fibers, as by carding, air laying, or the like. The exact weight of the fibrous web has not been found to be narrowly critical, although useful weights have been found within the range from about 0.2 to about 4.2 ounces per square yard (about 6.78 to about_{'}142.4 g/m²).

The web comprising a loose array of polyester/ polyethylene conjugate fibers is laid on an open mesh network surface and passed underforced air heating means. The forced heated air pushes the fibers in open areas of the mesh out of the plane of the fabric and fuses the polyethylene component of the conjugate fibers and form bonds at points of fiber-to-fiber contact. Forced heated air at a face velocity of at least 100ft./min. (0.51 m/s) is applied to a circular drum with a vacuum drawn at three- tenths inch (7.6 mm) of water within the drum. The exact temperatures employed will vary, depending upon the weight and bulk density of the web, and upon the dwell time employed in the heated zone. For instance, bonding temperatures within the range from about 130° to about 18o^{o}e., have been found satisfactory. Dwell times in the heated zone will usually vary from about 2 seconds to about 1 minute, and more normally will be from about 3 to about 10 seconds.

In an alternative embodiment of a method and apparatus of the present invention, an air permeable restraining belt 28 may be provided and carried along means 30 for causing said restraining belt to travel along with the open mesh network surface. The restraining belt compresses the web against the open mesh network creating a fabric as shown at 60 in Figure 4. The fabric has one surface 63 comprising puffed regions 64 wherein the fibers are bent out of the plane 65 of the fabric. The puffed regions have very low density. As shown especially in Figure 4A, the fabric also comprises densified regions 66 which extend between and around the puffed regions. The densification is caused by the compression of the web against the open mesh structure by the belt 28. The other surface of the fabric 68 formed next to the belt 28 is smooth.

In yet another alternative of the method and apparatus according to the present invention, the restraining belt may comprise an endless belt open mesh network. A fabric formed thereby is shown in Figure 5. The fabric shown generally at 70 comprises one face 72 which comprises puffed regions 74 wherein the fibers are puffed out of the plane 75 of the fabric, and densified regions 76 therebetween formed by the compression of the web against the open mesh network restraining belt. The fabric also comprises embossed type densification at least at surface 78 introduced by the open mesh network retraining belt. The emboss-type densification gives an embossed type pattern to the other surface 78. As shown in Figure 5A, the open mesh networks 16 and 28' had the same configuration and were in registry; however, the present invention contemplates different open mesh networks used as the moving surface and as the restraining belt and also contemplates the belts being used when they are not in registry creating a fabric wherein the other surface 78 has embossed type densified regions which do not coincide with the densified regions created by compressing the web against the open web structure moving surface.

The foregoing description and drawings are illustrative but are not to be taken as limiting. Other variations and modifications are possible without departing from the scope of the present invention.

## Claims

1. Process for making a nonwoven fabric having high bulk and low density comprising:
(a) superimposing a web comprising at least 10 percent conjugate fibers comprising a low melting point component on a moving open mesh network surface having open areas therein; and
(b) applying forced heated air to the exposed surface of the web to bend the fibers adjacent the open areas into the open areas and to heat fuse the low melting point component of the conjugate fibers to fibers in the web, forming a fabric with a patterned surface adjacent the open mesh network.

2. The process of Claim 1 further comprising the step of restraining the web against the open mesh network during the application of forced air.

3. The process of Claim 2 wherein said restraining means comprises another open mesh network.

4. The process of Claims 1, 2 or 3 wherein the web is cooled between the open mesh network and restraining means.

5. In an apparatus for forming and thermal bonding a fibrous web comprising conjugate fibers, said apparatus comprising a frame with a movable surface and means for forcing heated air onto the movable surface; the improvement comprising an open mesh network superimposed on the movable surface.

6. An apparatus as in Claim 5 further comprising an air permeable restraining belt and means for causing said restraining belt to travel along with the movable surface.

7. An apparatus as in Claim 5 or 6 wherein said open mesh network comprises an endless belt with means for causing said endless belt open mesh network to and from the movable surface.

8. A high loft, low density nonwoven fabric comprising at least 10 percent conjugate fibers comprising a low melting point component, said fabric comprising a patterned surface comprising a pattern of puffed regions of low density wherein the fibers are bent out of the plane of the fabric.

9. A nonwoven fabric as in Claim 8 further comprising densified regions between the puffs.

10. A nonwoven fabric as in Claim 9 or 10 further comprising an emboss type patterned other surface formed the emboss type densified regions formed in at least the other surface of the fabric.

## Patentansprüche

1. Verfahren zur Herstellung eines Faservliesstoffes von hoher Bauschigkeit und niedriger Dichte, welches Verfahren die folgenden Schritte umfaßt:
(a) das Auflegen einer Bahn mit einem Gehalt von wenigstens 10% an Konjugatfasern, welche eine Komponente mit niedrigem Schmelzpunkt enthalten, auf einer in Bewegung befindlichen offenmaschigen Netzwerksoberfläche, welche offene Bereiche darin aufweist; und
(b) das Beaufschlagen der exponierten Oberfläche der Bahn mit erhitzter Gebläseluft, um die neben den offenen Bereichen befindlichen Fasern in die offenen Bereiche hineinzubiegen und um die Komponente mit dem niedrigen Schmelzpunkt der Konjugatfasern mit Fasern in der Bahn warmzuverschweißen, unter Bildung eines Stoffes, der neben dem offenmaschigen Netzwerk eine gemusterte Oberfläche aufweist.

2. Verfahren nach Anspruch 1, welches weiterhin die Stufe des Zurückhaltens der Bahn gegen das offenmaschige Netzwerk während der Anwendung der Gebläseluft umfaßt.

3. Verfahren nach Anspruch 2, wobei das Rückhaltemittel ein anderes offenmaschiges Netzwerk umfaßt.

4. Verfahren nach Ansprüchen 1, 2 oder 3, wobei die Bahn zwischen dem offenmaschigen Netzwerk und dem Rückhaltemittel gekühlt wird.

5. Verbesserung einer Vorrichtung zum Formen und thermischen Binden einer Faserstoffbahn mit einem Gehalt an Konjugatfasern, welche Vorrichtung einen Rahmen mit einer beweglichen Oberfläche und Einrichtungen zum Beaufschlagen der beweglichen Oberfläche mit erhitzter Gebläseluft umfaßt; wobei die Verbesserung darin besteht, daß die Vorrichtung ein auf der beweglichen Oberfläche aufgelegtes, offenmaschiges Netzwerk umfaßt.

6. Vorrichtung nach Anspruch 5, welche weiterhin ein luftdurchlässiges Rückhalteband und Einrichtungen zum Führen dieses Rückhaltebandes gemeinsam mit der beweglichen Oberfläche umfaßt.

7. Vorrichtung nach Anspruch 5 oder 6, worin das offenmaschige Netzwerk ein Endlosband zusammen mit Einrichtungen umfaßt, welche dazu dienen, das Endlosband mit dem offenmaschigen Netzwerk zu der beweglichen Oberfläche hin und von dieser wieder wegzubewegen.

8. Hochvoluminöser Faservliesstoff von niedriger Dichte und mit einem Gehalt von wenigstens 10% an Konjugatfasern, welche eine Komponente mit einem niedrigen Schmelzpunkt enthalten, welcher Stoff eine gemusterte Oberfläche aufweist, welche Oberfläche ein Muster von aufgeblähten Bereichen von niedriger Dichte aufweist, in welchen Bereichen die Fasern aus der Ebene des Stoffes herausgebogen sind.

9. Faservliesstoff nach Anspruch 8, welcher weiterhin zwischen den aufgeblähten Bereichen verdichtete Bereiche aufweist.

10. Faservliesstoff nach Anspruch 9 oder 10, welcher weiterhin eine gemusterte andere Oberfläche vom geprägten Typus umfaßt, welche gemusterte Oberfläche durch verdichtete Bereiche vom geprägten Typus, die in wenigstens der anderen Oberfläche des Stoffes geformt sind, gebildet wird.

## Revendications

1. Procédé de fabrication de textile non tissé ayant un bouffant important et une faible densité qui comprend:
(a) la superposition d'une nappe comprenant au moins 10 pourcents de fibres complexes ayant un composant à bas point de fusion sur une surface à réseau de maille ouverte comportant des aires ouvertes; et
(b) l'application d'air chaud à ventilation forcée sur la surface exposée de la nappe pour courber les fibres adjacentes aux aires ouvertes dans les aires ouvertes et pour souder par fusion le composant à bas point de fusion des fibres complexes aux fibres de la nappe, de façon à former un textile à surface gaufrée adjacente au réseau à maille ouverte.

2. Procédé selon la revendication 1, comprenant en plus l'étape de maintien de la nappe contre un réseau à maille ouverte pendant l'application d'air sous ventilation forcée.

3. Procédé selon la revendication 2 dans lequel le moyen de maintien comprend un autre réseau à maille ouverte.

4. Procédé selon les revendications 1, 2 ou 3, dans lequel la nappe est refroidie entre le réseau à maille ouverte et le moyen de maintien.

5. Dans un appareil de fabrication et de soudage thermique d'une nappe de fibre comprenant des fibres complexes, ledit appareil comprenant un châssis avec une surface mobile et des moyens pour pulser de l'air chauffé sur la surface mobile; l'amélioration comprenant un réseau à maille ouverte superposé à la surface mobile.

6. Appareil selon la revendication 5, comprenant en outre une courroie de maintien perméable à l'air et des moyens pour entraîner ladite courroie de maintien le long de la surface mobile.

7. Appareil selon la revendication 5 ou 6, dans lequel ledit réseau à maille ouverte comprend une courroie sans fin avec des moyens permettant à ladite courroie sans fin à réseau à maille ouverte d'aller sur la surface mobile et de la quitter.

8. Textile non tissé de grand volume et de faible densité, comprenant au moins 10 poucents de fibres complexes, comportant un composant à bas point de fusion, ce textile comprenant une surface gaufrée qui comprend un réseau de zones expansées de faible densité dans lesquelles les fibres sont recourbées hors du plan du textile.

9. Texile non tissé selon la revendication 8, comprenant en plus des zones densifiées entre les zones expansées.

10. Textile non tissé selon la revendication 9 ou 10 comprenant une autre face à réseau de type gaufrage, formée par des régions densifiées sur au moins l'autre face du textile.
